

1

3,437,641  
**PROCESS FOR IMPROVING THE ACID DYE RECEPTIVITY OF POLYLACTAMS AND POLYLACTAM PRODUCTS SO PRODUCED**  
Jürgen Lenz, Obernburg, and Ernst Meyer, Erlenbach, Germany, assignors to Vereinigte Glanzstoff-Fabriken AG., Wuppertal-Elberfeld, Germany  
No Drawing. Filed Feb. 28, 1966, Ser. No. 530,374  
Claims priority, application Germany, Mar. 3, 1965,  
U 27,948  
Int. Cl. C08g 41/02  
U.S. CL. 260—78

10 Claims

## ABSTRACT OF THE DISCLOSURE

Process of improving the acid dye receptivity of polycaprolactam and the resulting product wherein there is homogeneously incorporated in the polycaprolactam a small amount of (a) a phosphoric acid ester or an alkyl or aryl phosphonic acid or an ester thereof, and (b) an alkylene polyamine. The product exhibits improved receptivity for acid dyes with a minimum reduction of its solution viscosity.

This invention relates to a process for improving the dye receptivity of polylactams for acid dyes, and more particularly, the invention is directed to a process of incorporating a combination of certain organic phosphorous compounds and amines into a fiber-forming polylactam, especially polycaprolactam, so as to obtain a product which is easily spun into textile fibers and which can be dyed in an improved manner with acid dyes.

It is known that the dye receptivity of fiber-forming polyamides for acid dyes can be improved if the polyamide is initially treated so as to contain an increased number of amino end groups. One method of achieving this result has been to add free amines to the polyamide-forming initial materials prior to polycondensation. Suitable amines which have been suggested for this purpose include aliphatic monoamines or diamines and heterocyclic amines. Where the polyamide is obtained by polycondensation of dicarboxylic acids and diamines, e.g., in the preparation of polyhexamethylene adipamide, only a small excess of the above-noted free amines is necessary. On the other hand, a considerably greater amount of the free amines must be added when using lactams as the monomers in the formation of a fiber-forming polyamide. The polyamides which are produced according to this known process and which show a higher number of amino groups are not fully satisfactory because they are more difficult to spin into filaments or fibers. For example, if one wishes to obtain an appreciable improvement in dyeability and correspondingly adds larger amounts of the amine, the resulting polyamide has a substantially lower viscosity and the molten polyamide tends to drip during spinning, so that a spinning of the polyamide melt into filaments is no longer practical.

According to another known process, this defect in the polyamide caused by the addition of the amine is supposed to be avoided by adding phosphorous compounds to the polyamide prior to spinning. Suitable phosphorous compounds suggested for this purpose are hypophosphites of alkali and alkaline earth metals as well as those of zinc, cadmium, manganese, aluminum and tin, and also salts

2

of phosphinic acid. According to still another known process, the dye receptivity of polyamides is supposed to be improved by the addition of alkyl- or aryl-phosphinic acids or their amine salts. It has become apparent that the addition of such compounds, particularly the amine salts of phosphinic acids, results in an appreciable improvement of the dye receptivity whereas the metal salts of phosphinic acid do not have any effect. In any case, the known processes are restricted to polyamides prepared from dicarboxylic acids and diamines. If one attempts to apply these additives to polyamides formed from lactams, then it has been found that only a slight and unimportant improvement in dye receptivity is possible.

One object of the present invention is to provide a process whereby a substantially improved acid dye receptivity can be imparted to a fiber-forming polylactam without impairing the subsequent spinning of the polymer into filaments.

Another object of the invention is to provide a process for improving the receptivity of a fiber-forming polylactam for acid dyes by using a novel combination of additives which can be easily incorporated into the polylactam either before or during polycondensation of the lactam monomer or subsequently to the polylactam before it is spun into textile fibers.

These and other objects and advantages of the invention will become more apparent upon consideration of the following detailed specification.

It has now been found, in accordance with the invention, that the foregoing objects can be achieved by homogeneously incorporating into a fiber-forming polylactam: (a) about 0.05 to 3% by weight, preferably about 0.1 to 2% by weight, of an organic phosphorous compound selected from the group consisting of phosphoric acid esters and alkyl and aryl phosphonic acids and their esters; and (b) about 0.01 to 1% by weight, preferably 0.02 to 0.5% by weight, of a polyamine of the formula



wherein  $m$  represents an integer of 0 to 3,  $n$  represents an integer of 2 to 6 and the sum of  $m$  and  $n$  is not more than 6.

The term "dye receptivity" is employed herein with reference to the ability of the polymer fiber to absorb or take up an acid dye during any conventional method of dyeing. The polylactams which are improved by the process of this invention are well known fiber-forming polymers containing recurring  $-\text{NHCO}-$  groups connected by an alkylene group in the polymer chain. Polycaprolactam, sometimes referred to as "nylon 6," is most often used for commercial textiles, and the production of the polyamide from the monomeric lactam, such as epsilon-caprolactam is quite well known and requires no further explanation.

The two essential additives of the invention, i.e., the organic phosphorous compound and the polyamine can be introduced and incorporated into the polycaprolactam at any point prior to spinning filaments or fibers therefrom, under conditions which ensure an homogeneous mixture of the polymer and the additives, e.g., by thorough mixing during polycondensation or by kneading and homogenizing the additives with the molten polymer in an extruder or similar mixing device. Thus, the additives may be introduced before the polycondensation of the lactam

monomer or at any suitable time during the polycondensation reaction. Moreover, it is possible to admix the two essential components of the invention with the polylactam product, which is in the form of cuttings, granules or small pellets at a point prior to spinning, e.g., by panniering the cuttings or otherwise surface coating the polymer particles. Thereafter, the organic phosphorous compound and the polyamine are homogeneously mixed with the polylactam by any conventional method, e.g., by re-extruding the treated material in a screw extruder or even in a mixing section just preceding the melt spinning operation.

As the organic phosphorous compound employed as component (a) in the process of the invention, it is particularly desirable to employ those compounds of the formula



or



in which X stands for aryl or alkyl, preferably phenyl and lower alkyl such as methyl, ethyl, propyl or butyl, X' stands for aryl such as phenyl, aralkyl such as benzyl or lower alkyl, i.e., alkyl of 1 to 4 carbon atoms, and Y stands for hydrogen, aryl such as phenyl, or lower alkyl of 1 to 4 carbon atoms. Specific organic phosphorous compounds suitable for the purposes of the invention can be listed as follows:

Tributyl phosphate  
 Methanephosphonic acid dimethyl ester  
 Ethanephosphonic acid diethyl ester  
 Phenyl-methanephosphonic acid diethyl ester  
 Tripropylphosphate  
 Triethylphosphate  
 Trimethylphosphate  
 Triphenylphosphate  
 Phenyl-methanephosphonic acid dibutyl ester  
 Phenyl-methanephosphonic acid diphenyl ester  
 Benzenephosphonic acid  
 Benzenephosphonic acid dibutyl ester  
 Benzenephosphonic acid diphenyl ester  
 Ethanephosphonic acid

As to the amine component (b), the best results are achieved in accordance with the invention by using a compound of the formula



in which p stands for an integer of 2 to 4, i.e., diethylene triamine, triethylene tetramine and tetraethylene pentamine. In addition, the following specific polyamines are also suitable:

Hexamethylene diamine  
 Pentamethylene diamine  
 Tetramethylene diamine  
 Trimethylene diamine  
 Ethylene diamine  
 Dipropylene diamine  
 Tripropylene tetramine  
 Tetrapropylene pentamine  
 Dibutylene triamine  
 Tributylene tetramine  
 Dipentylene triamine

If a phosphoric or phosphonic acid ester of the invention is added alone for increasing the acid dye receptivity of the polylactam, then some increase in dyeability does take place—although it is proportionately less than that achieved by the process of the invention. Even this effect cannot be achieved with the known phosphinic acids or phosphinic acid derivatives when they are used with a polylactam.

On the other hand, even when using the organic phosphorous compounds of the present invention, the acid dye receptivity cannot be further increased simply by the addition of larger amounts of this component because the viscosity of the polylactam is then simultaneously reduced. However, if one introduces a mixture of the phosphoric or phosphonic acid ester together with a small amount of the polyamine as the second component, within the proportions defined by the invention, then the acid dye receptivity of the polylactam increases quite sharply in a very surprising manner. Although the amines just as the organic phosphorous compounds cause a lowering of the viscosity, it has been found that a definite synergistic effect takes place with the dye receptivity increasing much more rapidly than any accompanying decrease in viscosity. Thus, one can obtain an optimum improvement of dye affinity or receptivity with the least possible reduction of viscosity by the suitable selection of the phosphorous compounds and amines as well as by choosing appropriate amounts of these compounds within the prescribed limits of the invention. In this respect, the preferred polyethylene polyamines as noted above offer the greatest advantage because they yield a very substantial increase in dye absorption even when using quite small amounts, and these small amounts of the polyamine have only a slight influence on the viscosity.

Especially favorable results are achieved according to the invention if the organic phosphorous compounds and amines are added to the completely condensed polylactam prior to spinning into filaments. When the process of the invention is carried out in this manner, there is practically no influence on the viscosity of the polymer. Surprisingly, however, the improvement in the acid dye receptivity is considerable. This result was not at all expected because it had been previously assumed that in order to increase the number of amino end groups, it would be absolutely essential to introduce any additives—especially amines—into the initial monomeric materials.

The invention is further illustrated by without being limited to the following examples. In these examples as well as in the appended claims and elsewhere in this specification, the percentages of the phosphorous and amine compounds are by weight with reference to the particular lactam or polylactam which is being treated. The solution viscosity is measured in each instance by measuring the flow rate of a 1% solution of the polylactam in formic acid. Extinction values are obtained by conventional measurement of the dye solutions.

#### EXAMPLE I

While caprolactam is being polycondensed in a conventional manner, there is added to the fluid monomer 1% by weight of ethanephosphonic acid diethyl ester and 0.3% by weight of diethylene triamine. The resulting polyamide has a solution viscosity of 2.05 and has good spinning qualities. In order to ascertain the dyeing improvement which has been achieved, filaments of the polyamide containing the above named additives are dyed together with polyamide filaments which contain no additives in the same bath with the acid dye Anthralan Blue B. The dye absorbed from the bath by the two filament samples is thereafter completely extracted with a pyridine-water mixture. The extinction of both dye solutions is measured, and amounted to a proportion of 1:3.8 (polyamide without additives:polyamide+phosphorous compound+amine).

As described in the above example, further tests were

carried out while changing the additive compounds or their proportions as summarized in the following table:

the solution viscosity of the additive-containing cuttings compared to the normal polyamide is somewhat lower,

| Test Number:      | Additives                                          | Percent by weight | Solution viscosity | Extinction proportion |
|-------------------|----------------------------------------------------|-------------------|--------------------|-----------------------|
| 1.                | {Ethanephosphonic diethyl ester.....               | 1.0               | 2.05               | 1:3.80                |
|                   | {Diethylene triamine.....                          | 0.3               |                    |                       |
| 2.                | {Ethanephosphonic acid diethyl ester.....          | 1.0               | 1.98               | 1:9.20                |
|                   | {Diethylene triamine.....                          | 0.4               |                    |                       |
| 3.                | {Ethanephosphonic acid diethyl ester.....          | 0.1               | 2.14               | 1:2.34                |
|                   | {Hexamethylene diamine.....                        | 0.3               |                    |                       |
| 4.                | {Ethanephosphonic acid diethyl ester.....          | 0.5               | 2.15               | 1:2.27                |
|                   | {Hexamethylene diamine.....                        |                   |                    |                       |
| 5.                | {Ethanephosphonic acid diethyl ester.....          | 0.7               | 2.14               | 1:3.05                |
|                   | {Hexamethylene diamine.....                        | 0.3               |                    |                       |
| 6.                | {Ethanephosphonic acid diethyl ester.....          | 1.0               | 2.06               | 1:2.93                |
|                   | {Hexamethylene diamine.....                        | 0.3               |                    |                       |
| 7.                | {Ethanephosphonic acid diethyl ester.....          | 1.5               | 1.90               | 1:2.83                |
|                   | {Hexamethylene diamine.....                        |                   |                    |                       |
| 8.                | {Ethanephosphonic acid diethyl ester.....          | 2.0               | 1.90               | 1:2.95                |
|                   | {Hexamethylene diamine.....                        | 0.3               |                    |                       |
| 9.                | {Ethanephosphonic acid diethyl ester.....          | 0.5               | 2.05               | 1:3.30                |
|                   | {Hexamethylene diamine.....                        |                   |                    |                       |
| 10.               | {Ethanephosphonic acid diethyl ester.....          | 1.0               | 1.99               | 1:4.35                |
|                   | {Hexamethylene diamine.....                        |                   |                    |                       |
| 11.               | {Ethanephosphonic acid diethyl ester.....          | 1.5               | 1.89               | 1:4.80                |
|                   | {Hexamethylene diamine.....                        | 0.4               |                    |                       |
| 12.               | {Methanephosphonic acid dimethyl ester.....        | 0.75              | 2.05               | 1:3.31                |
|                   | {Diethylene triamine.....                          | 0.3               |                    |                       |
| 13 <sup>1</sup> . | {Phenyl-methanephosphonic acid dimethyl ester..... | 2.5               | 2.01               | 1:1.65                |
| 14 <sup>1</sup> . | None.....                                          |                   | 2.16               |                       |
| 15.               | {Ethanephosphonic acid diethyl ester.....          | 1.0               | 2.00               | 1:4.56                |
|                   | {Triethylene tetramine.....                        | 0.4               |                    |                       |
| 16.               | {Ethanephosphonic acid diethyl ester.....          | 1.0               | 2.00               | 1:5.05                |
|                   | {Tetraethylene pentamine.....                      | 0.5               |                    |                       |

<sup>1</sup> Comparative tests.

## EXAMPLE II

Dried polycaprolactam cuttings ready for spinning with a solution viscosity of 2.55 are mixed in a tumbler drier successively with 0.3% by weight of hexamethylene diamine and 1% by weight of tributyl phosphate. Thereafter, these cuttings are regranulated in an extruder. After the regranulation, the modified polycaprolactam exhibits a solution viscosity of 2.53. The cuttings are then spun and the resulting filaments dyed as described in Example I. By measuring the extinction proportion of the dyestuff extracted from each of the filament samples, the dyeing improvement of the modified polyamide by comparison with the unmodified polyamide is ascertained. The extinction proportion in this case amounts to 1:2.63 (polyamide without additive:polyamide+phosphorous compound+amine).

As described in Example II above, further tests are carried out with changes in the compounds or additive amounts as summarized in the following table:

30 an increase of the viscosity occurs in the spinning process. In this manner, therefore, a very high viscosity of the finished filaments is assured. The addition of the amine, on the other hand, acts as a viscosity stabilizer and reduces the filament viscosity during the spinning process, thereby preventing an undesirably large increase in the solution viscosity. Also, this effect has proven to be certain as shown in the following tests.

## EXAMPLE III

40 The tests of this example are carried out in order to show that a polyamide of caprolactam containing phosphonic acid esters during the spinning also is subject to a high degree of after-condensation, even if the cuttings contain amines as the second additive.

45 Polyamide cuttings which contain the additives set forth in Table III, are spun with an extruder spinning machine at a temperature of 275° C. Samples are taken from the initial cuttings and the spun filaments and the solution viscosities determined in the same manner as

| Test Number:     | Additives                   | Percent by weight | Solution viscosity of cuttings | Extinction proportion |
|------------------|-----------------------------|-------------------|--------------------------------|-----------------------|
| 1.               | {Tributyl phosphate.....    | 1.0               | 2.53                           | 1:2.63                |
|                  | {Hexamethylene diamine..... | 0.3               |                                |                       |
| 2.               | {Tributyl phosphate.....    | 2.0               | 2.47                           | 1:2.91                |
|                  | {Hexamethylene diamine..... | 0.3               |                                |                       |
| 3 <sup>1</sup> . | Tributyl phosphate.....     | 1.0               | 2.62                           | 1:2.13                |
| 4 <sup>1</sup> . | Hexamethylene diamine.....  | 0.3               | 2.42                           | 1:2.02                |

<sup>1</sup> Comparative tests.

A further advantage of the process according to the invention is to be seen in the fact that during the spinning of the polyamide the added phosphorous compounds cause a considerable after-condensation, so that even if

60 in Example I. Through the high increase of the solution viscosity during the spinning, the effect of the phosphonic acid ester and amine added during the polymerization in lowering the solution viscosity is substantially reduced.

## TABLE III

| Test Number: | Additives                                 | Percent by weight | Solution viscosity of cuttings | Solution viscosity of the spun filaments |
|--------------|-------------------------------------------|-------------------|--------------------------------|------------------------------------------|
| 1.           | Ethanephosphonic acid diethyl ester.....  | 0.7               | 2.06                           | 2.91                                     |
| 2.           | Hexamethylene diamine.....                | 0.3               | 2.13                           | 2.27                                     |
| 3.           | {Ethanephosphonic acid diethyl ester..... | 1.8               |                                |                                          |
|              | {Hexamethylene diamine.....               | 0.3               | 1.90                           | 2.35                                     |
| 4.           | {Ethanephosphonic acid diethyl ester..... | 1.0               |                                |                                          |
|              | {Diethylene triamine.....                 | 0.3               | 2.15                           | 2.62                                     |

The invention is hereby claimed as follows:

1. A process for improving the receptivity of a fiber-forming polycaprolactam for acid dyes which comprises: homogeneously incorporating into said polycaprolactam:
- about 0.05 to 3% by weight, with reference to the polycaprolactam, of an organic phosphorous compound selected from the group consisting of phosphoric acid esters and alkyl and aryl phosphonic acids and their esters, and
  - about 0.01 to 1% by weight, with reference to the polycaprolactam, of a polyamine of the formula



wherein  $m$  represents an integer of 0 to 3,  $n$  represents an integer of 2 to 6 and the sum of  $m$  and  $n$  is not more than 6.

2. A process as claimed in claim 1 wherein (a) is used in an amount of about 0.1 to 2% by weight and (b) is used in an amount of about 0.02 to 0.5% by weight.

3. A process as claimed in claim 1 wherein component (a) is a phosphoric acid ester of the formula



wherein X represents a substituent selected from the group consisting of lower alkyl and phenyl.

4. A process as claimed in claim 1 wherein component (a) is a compound of the formula



wherein X' represents a substituent selected from the

35 260-78; 8-55

group consisting of lower alkyl, phenyl and benzyl and Y represents a substituent selected from the group consisting of hydrogen, lower alkyl and phenyl.

5. A process as claimed in claim 1 wherein component (b) is a compound of the formula



wherein  $p$  represents an integer of 2 to 4.

6. A process as claimed in claim 1 wherein component (b) is hexamethylene diamine.

7. A process as claimed in claim 1 wherein component (a) is ethanephosphonic acid diethyl ester.

8. A process as claimed in claim 1 wherein component (a) is methanephosphonic acid dimethyl ester.

- 15 8. A process as claimed in claim 1 wherein component (a) is tributyl phosphate.

- 10 10. The polylactam product obtained by the process of claim 1.

#### References Cited

##### UNITED STATES PATENTS

|           |        |                 |       |        |
|-----------|--------|-----------------|-------|--------|
| 2,241,322 | 5/1941 | Hanford         | ----- | 260-78 |
| 2,510,777 | 6/1950 | Gray            | ----- | 260-78 |
| 2,557,808 | 6/1951 | Walker          | ----- | 260-78 |
| 2,904,536 | 9/1959 | Reith           | ----- | 260-78 |
| 3,296,215 | 1/1967 | Crovatt         | ----- | 260-78 |
| 3,296,216 | 1/1967 | Snooks          | ----- | 260-78 |
| 3,300,448 | 1/1967 | Gauthier et al. | ----- | 260-78 |

30 WILLIAM H. SHORT, Primary Examiner.

H. D. ANDERSON, Assistant Examiner.

U.S. CL. X.R.

**U.S. DEPARTMENT OF COMMERCE  
PATENT OFFICE  
Washington, D.C. 20231**

**UNITED STATES PATENT OFFICE  
CERTIFICATE OF CORRECTION**

Patent No. 3,437,641

April 8, 1969

Jürgen Lenz et al.

It is certified that error appears in the above identified patent and that said Letters Patent are hereby corrected as shown below:

In the heading to the printed specification, line 10, "U 27,948" should read -- V 27,948 --.

Signed and sealed this 21st day of April 1970.

(SEAL)

Attest:

Edward M. Fletcher, Jr.

Attesting Officer

**WILLIAM E. SCHUYLER, JR.**

Commissioner of Patents